

1

3,810,760

## PHOTOGRAPHIC DRY COPYING PROCESS WITH ACYLACETONITRILE

Helmut Kampfer and Hans Ohlschlager, Cologne, Anita von Konig, Leverkusen, and Johannes Gotze, Bergisch Neukirchen, Germany, assignors to Agfa-Gevaert Aktiengesellschaft, Leverkusen, Germany  
No Drawing. Filed Feb. 10, 1972, Ser. No. 225,314  
Claims priority, application Germany, Feb. 11, 1971,

P 21 06 577.0

Int. Cl. G03c 1/40, 1/52, 5/54

U.S. Cl. 96—29 D

10 Claims

### ABSTRACT OF THE DISCLOSURE

Photographic images are produced by (1) imagewise exposing a light-sensitive layer containing at least one sensitizing dye from the class of the neutrostyryl dyes, the merocyanines or a cyanine dye containing a halogen substituted benzene ring or a heterocyclic ring derived from selenazol, a compound of the guanidine or biguanide series and an image-producing reducing acylacetonitrile derivative which is transferable at temperatures between 80 and 200° C., whereby, at the exposed areas the image-producing reducing compound is converted to a non-transferable compound, (2) bringing the exposed layer into contact with an image-receiving layer which contains compounds capable of reacting with the image-producing compound transferred from the unexposed areas of the light-sensitive layer to form colored products and (3) heating the layers while in contact with each other to a temperature of between 80 and 200° C. to produce a visible image.

The invention is concerned with a photographic dry copying process and a light-sensitive material for carrying out this process.

Photographic processes that produce copies by dry methods are known per se. These processes make use of materials containing light- or heat-sensitive layers which are imagewise exposed or heated thus causing a photochromic reaction which bring about the formation of the image.

The known light-sensitive materials of the type mentioned above, from which negative images can be produced, have, however, several disadvantages. For example, their light sensitivity—especially in the visible region of the spectrum—is unsatisfactory so that too lengthy copying times are required and the reproduction of colored originals present difficulties. Moreover, the finished images still remain sensitive to light and their stabilization with respect to daylight can, in general, be achieved only by a quite complicated after-treatment.

Processes for the production of copies are also known in which a light-sensitive coating, which contains a light-sensitive compound and an image-producing compound transferable to an image-receiving layer, is exposed to the image so that at the exposed areas the image-producing compound is converted to a non-transferable compound; the exposed layer is brought into contact with an image-receiving layer which contains compounds that react with the image-producing compound to form a dye and the layer while in contact with each other are heated to a temperature at which the image-producing compound is transferred from the exposed areas of the light-sensitive layer to the image-receiving layer.

To these processes belong, for example, the so-called heat-development processes in which light-sensitive materials having a silver halide emulsion layer which contains a photographic developer are employed. After exposure, they are developed by heating in contact with an image-receiving layer which contains substances capable of yielding a dye by reaction with the developer. When heated,

2

the developer is transferred from the unexposed areas of the light-sensitive coating to the image-receiving layer to produce a dye image.

A disadvantage of these known heat development or developer-sublimation processes is the unsatisfactory storage of the silver halide emulsion layer containing the developer caused by the presence of substances that increase the residual moisture of the layers, such as salts which form hydrates or glycols, and by the increased sensitivity to oxidation of most developers in these slightly hardened or unhardened emulsion layers with high residual moisture.

The process described in USP No. 3,094,417 is also of this type. In this process light-sensitive emulsions are employed containing a transferable compound and a dye. On exposure the transferable compound, e.g. 4-methoxy-1-naphthol is converted to a nontransferable product. By subsequent heating, this compound can be transferred from the unexposed areas to an image-receiving layer where it reacts with a silver salt, e.g. silver behenate to give a positive silver image.

A similar process has been described in OLS 2,010,837 in which acetoacetonitrile derivatives which can be inactivated by light and which are capable of reacting with a silver salt are employed.

All these processes have the disadvantage that the sensitivity of the emulsion layers is often low or the stability of the material is limited or that the production of copies having a high gamma and high contrast presents difficulties.

It is among the objects of the present invention to provide photographic dry copying processes and light-sensitive materials suitable for such processes which are very sensitive to light and stable and which contain dyes which render the material sensitive to every required region of the spectrum and which allow the production of both multicolored and black images.

We now have found a process for the production of photographic images comprising the steps of (1) imagewise exposing a light-sensitive layer containing at least one sensitizer of the class of neutrostyryl dyes, merocyanines or a cyanine dye containing a halogen substituted benzene ring or a heterocyclic ring derived from selenazol, a compound of the guanidine or biguanide series and an image-producing reducing agent of the acylacetonitrile series, being transferable at temperatures in the range of from 80 to 200° C. to an image-receiving layer, whereby at the exposed areas the image-producing reducing agent is converted to a non-transferable compound, (2) bringing the exposed layer into contact with an image-receiving layer which contains a compound capable of reacting with the reducing agent transferred from the unexposed areas to form colored products and (3) heating the layers while in contact at a temperature in the range of from 80 to 200° C. to produce a visible image in the image-receiving layer.

The light-sensitivity of the layer is highly increased by the addition of at least one of the guanidine or biguanide derivatives.

Compounds of the following formula have proved to be particularly suitable:



65 wherein

R<sup>1</sup>=hydrogen or aryl, especially a radical of the phenyl series, the aryl group or especially the phenyl ring may, in any position but preferably in the ortho or para position, be substituted by preferably alkyl or alkoxy, both with preferably up to 3 C-atoms, halogen, such as fluorine, chlorine, bromine or iodine, but also by other

substituents such as carboxyl, esterified carboxyl, sulfo, sulfonamide or esterified sulfo groups;

$R^2$ =aryl, preferably, a radical of the phenyl series, where the aryl group or the phenyl ring may be substituted as described under  $R^1$ , or a group of the formula



where  $R^1$  has the meaning stated above.

*o*-Tolylbiguanide, 1,3-diphenylguanidine and 1,3-di-*o*-tolylguanidine are particularly suitable.

Acylacetonitrile derivatives of the following general formula are suitable as image-producing reducing agents transferable in the temperature range from 80 to 200° C.:



where

$R^3$ =(1) alkyl with up to 5 C-atoms, preferably methyl or ethyl, (2) alkoxy or alkoxy carbonyl with preferably up to 5 C-atoms, (3) aryl or substituted aryl, especially a radical of the phenyl series, which may be substituted for example with alkyl or alkoxy, both with preferably not more than 3 C-atoms, or halogen, such as fluorine, chlorine, bromine or iodine as well as by other substituents like esterified carboxyl, or (4) aralkyl, especially benzyl or phenylethyl;

$R^4$ =(1) aryl, in particular a group of the phenyl series, 35  
which may be substituted, for example, by halogen,  
such as fluorine, chlorine, bromine or iodine; phenyl,  
phenoxy, alkyl or alkoxy, both preferably with not more  
than 3 C-atoms, or (2) heterocyclic groups, such as  
furyl, pyridyl or thiényl. 40

Suitable compounds are contained in Table 1:

TABLE 1

| Nitrile number | R <sup>1</sup> -CO- | R <sup>4</sup>            |
|----------------|---------------------|---------------------------|
| 1              | Acetyl              | 4-methoxyphenyl.          |
| 2              | do                  | Phenyl.                   |
| 3              | do                  | 3-fluorophenyl.           |
| 4              | do                  | 3-methylphenyl.           |
| 5              | do                  | 4-methylphenyl.           |
| 6              | do                  | 4-phenylphenyl.           |
| 7              | do                  | 4-chlorophenyl.           |
| 8              | do                  | 3,4-dimethoxyphenyl.      |
| 9              | do                  | 4-bromophenyl.            |
| 10             | do                  | 2,5-dichlorophenyl.       |
| 11             | do                  | 4-iodophenyl.             |
| 12             | do                  | 3-chlorophenyl.           |
| 13             | do                  | 3,4,5-trimethoxyphenyl.   |
| 14             | Propionyl           | Phenyl.                   |
| 15             | Acetyl              | 2-furyl.                  |
| 16             | Benzoyl             | Phenyl.                   |
| 17             | Acetyl              | 3-pyridyl.                |
| 18             | 4-methoxybenzoyl    | Phenyl.                   |
| 19             | Acetyl              | 2-thienyl.                |
| 20             | do                  | 3,4-methylenedioxyphenyl. |
| 21             | Ethoxycarbonyl      | Phenyl.                   |

Compounds of the following types are suitable as sensitizers:

**(A) Neutrostyryl dyes of the general formulae**



where

Q=



$R^5$  = cyan,  $=CO-R^9$ ,  $=CO-N(R^9)_2$ ,  $=COOR^9$

$R^6 = R^9$  or  $-O-R^9, -N(R^9)_2$

$R^5$  and  $R^6$  together may also represent the members necessary for completing of an iso- or heterocyclic ketomethylene ring; these can be those rings that are conventional in cyanin chemistry such as those of the rhodanin series, like 3-ethylrhodanine, 3-allylrhodanine and 3-cyclohexylrhodanine, those of the 2-thio-2,4-oxazolidindione series like 3-ethyl-2-thio-2,4-oxazolidindione, those of the thiohydantoin series like 1,3-dimethyl-2-thiohydantoin and 1 - methyl-3-phenyl-2-thiohydantoin, those of the barbituric acid or thiobarbituric acid series like 1,3-diethyl-thiobarbituric acid and 1,3-diphenylthiobarbituric acid, those of the isoxazolone, oxindole, 2-thio-2,5-thiazolidindione, or the 2,4-imidazolidindione series or the ketomethylene compounds of the following structural formulae:



R<sup>7</sup>=hydrogen or nitro

$R^8$ =hydrogen,  $-\text{O}-R^9$ ,  $-\text{S}-R^9$ ,  $-\text{N}(R^9)_2$

5 R<sup>9</sup>=a saturated or olefinically unsaturated aliphatic group with preferably not more than 6 C-atoms, which can be substituted with, for example, phenyl, hydroxyl, halogen, such as chlorine or bromine, amino, carboxyl, sulfo or aryl, such as phenyl or naphthyl;

60  $Z^1, Z^2$ =hydrogen, alkyl preferably with not more than 3 C-atoms or alkoxy carbonyl preferably with not more than 4 C-atoms;  $Z^1$  and  $Z^2$  may also represent methylene groups forming part of a 5- or 6-membered ring;  $n=0, 1$  or 2

65 X=oxygen or sulfur.

The heterocyclic rings containing aryl groups may, if desired, contain further substituents such as further alkyl groups preferably with not more than 3 C-atoms, such as methyl or ethyl, halogen such as chlorine, bromine or iodine or the trifluoromethyl group, hydroxyl, alkoxy preferably with not more than 3 C-atoms such as methoxy or ethoxy, alkoxy carbonyl, hydroxyalkyl, alkylthio, aryl such as phenyl or aralkyl such as benzyl, amino, substituted amino and so on.

For example, the following compounds are suitable:







The dyes to be used in accordance with the invention are easily obtained by condensation of ketomethylene compounds with corresponding aldehydes in solvents such as alcohol, pyridine or glacial acetic acid, if desired with addition of a base like triethylamine or piperidine.

The preparation of the dyes A 7 and A 26 is described in detail below:

### Dye A 7

2.5 ml. of a 50% aqueous solution of sodium hydroxide were added to a solution of 4.0 g. o-hydroxycinnamaldehyde-O-acetic acid and 1.0 g. cyclohexanone in 50 ml. alcohol. After standing 30 minutes at room temperature, the mixture was acidified with dilute hydrochloric acid, the dye was removed by suction and recrystallized from chloroform/methanol. 2.4 g., M.P. 264-266° C. (under decomposition).

### Dye A 26

2.0 g. of 1,3-diethylthiobarbituric acid were heated 30 minutes on the steam bath with 1.7 g. 4-dimethylamino-cinnamaldehyde in 50 ml. alcohol. After cooling, the dye was removed by suction and recrystallized from chloroform/methanol. 3.3 g., M.P. 212-214° C.

(B) Halogen and/or selenium containing polymethin dyes of the general formulae:



where

Hal=Cl, Br or I;

R<sup>10</sup>=(1) a saturated or unsaturated aliphatic group with preferably not more than 6 C-atoms which may contain substituents such as halogen or phenyl, hydroxyl, amino, carboxyl, sulfo, sulfamoyl, carbamoyl, alkoxy-carbonyl, alkoxy, carboxyalkyl, sulfato or thiosulfato groups; (2) cycloalkyl such as cyclohexyl; or (3) aryl, especially a group of the phenyl series;

R<sup>11</sup>=hydrogen, alkyl with preferably not more than 3 C-atoms, aryl, such as phenyl, or cycloalkyl, such as cyclohexyl;

R<sup>12</sup>, R<sup>13</sup>=the same or different, namely hydrogen or hydroxyl, where however at least one of R<sup>12</sup> and R<sup>13</sup> is a hydroxyl group;

R<sup>14</sup>=hydrogen, alkyl or alkoxy with preferably not more than 5 C-atoms, halogen, especially chlorine, bromine or iodine, a trifluoromethyl group or aryl, especially a phenyl group;

R<sup>15</sup>=aryl such as phenyl, a heterocyclic ring such as thienyl or furyl which may also be substituted; X<sub>1</sub>=the ring members required for completing a benzene or naphthalene ring containing—if Y is different from Se—at least one halogen such as chlorine, bromine or iodine or a trifluoromethyl group, e.g. for the completion of a 5-iodobenzthiazole, 5-iodobenzselenazole, 6-iodobenzthiazole, 6-bromobenzthiazole, 5-bromo-benzoxazole or a 5-iodobenzoxazole ring and so on;

5 Z<sup>3</sup>, Z<sup>4</sup>=hydrogen, alkyl with preferably not more than 3 C-atoms or alkoxy carbonyl groups with preferably not more than 4 C-atoms; Z<sup>3</sup> and Z<sup>4</sup> can also be methylene groups necessary for completing a 5- or 6-membered ring;

10 Y=O, S, Se, —CH=CH, >N-alkyl, the alkyl having preferably up to 5 C-atoms, >N-aryl, in particular >N-phenyl;

Anion=any anion such as halide, e.g. chloride, bromide or iodide, perchlorate, sulfate, methyl sulfate, p-toluenesulfate; the anion is omitted if R<sup>10</sup> contains an acid group in the anionic form so that a betaine is present; n=0, 1 or 2;

D=the members of a ring necessary for completing an iso- or heterocyclic ketomethylene ring; these are the ketomethylene rings usual in cyanine chemistry, such as those of the rhodanine series like 3-ethylrhodanine, 3-allylrhodanine, 3-cyclohexylrhodanine, those of the 2-thio-2,4-oxazolidindione series like 3-ethyl-2-thio-2,4-oxazolidindione, those of the thiohydantoin series like 1,3-dimethyl-2-thiohydantoin, 1-methyl-3-phenyl-2-thiohydantoin, those of the barbituric acid or thiobarbituric acid series like 1,3-diethyl-thiobarbituric acid, 1,3-diphenylthiobarbituric acid, those of the isoxazolone, oxindole, 2-thio-2,5-thiazolidindione, 2,4-imidazolidindione series or the ketomethylene rings indicated by the following structural formulae:



Q=the members required for completion of 5- or 6-membered heterocyclic ring; the heterocyclic group may contain a fused benzene or naphthalene ring and further substituents; these are the heterocyclics conventional in cyanine chemistry such as those of the thiazole series (e.g. thiazole, 4-methylthiazole, 5-methylthiazole, 4,5-dimethylthiazole, 4-phenylthiazole, 5-phenylthiazole, 4,5-diphenylthiazole, etc.), those of the benzthiazole series (e.g. benzthiazole, 4-chlorobenzthiazole, 5-chlorobenzthiazole, 6-chlorobenzthiazole, 7-chlorobenzthiazole, 6-bromobenzthiazole, 5-iodobenzthiazole, 6-iodobenzthiazole, 4-methylbenzthiazole, 5-methylbenzthiazole, 6-methylbenzthiazole, 5,6-dimethylbenzthiazole, 4-phenylbenzthiazole, 5-phenylbenzthiazole, 6-phenylbenzthiazole, 5-hydroxybenzthiazole, 6-hydroxybenzthiazole, 4-methoxybenzthiazole, 5-methoxybenzthiazole, 6-methoxybenzthiazole, 5-ethoxybenzthiazole, 6-ethoxybenzthiazole, 5,6-dimethoxybenzthiazole, 5,6-methylenedioxobenzthiazole, 5-diethylaminobenzthiazole, 5-diethylaminobenzthiazole, 5-carboxybenzthiazole, 5-sulfobenzthiazole, tetrahydrobenzthiazole, 7-oxotetrahydrobenzthiazole etc.), those of the naphthothiazole series (e.g. naphtho(1,2-d)thiazole, naphtho(2,1-d)thiazole, 5-methoxynaphtho(2,1-d)thiazole, 5-ethoxynaphtho(2,1-d)thiazole, 7-methoxynaphtho(2,1-d)thiazole, 8-methoxynaphtho(1,2-d)thiazole etc.), those of the selenazole series (for example 4-methylselenazole

or 4-phenylselenazole), those of the benzoselenazole series (for example benzoselenazole, 5-chlorobenzoselenazole, 5,6-dimethylbenzoselenazole, 5-hydroxybenzoselenazole, 5-methoxybenzoselenazole, tetrahydrobenzoselenazole etc.), those of the naphthoselenazole series (for example naphtho(1,2-d)selenazole or naphtho(2,1-d)selenazole), those of the oxazole series (for example oxazole, 4-methyloxazole, 4-phenyloxazole, 4,5-diphenyloxazole etc.), those of the benzoxazole series (for example benzoxazole, 5-chlorobenzoxazole, 6-chlorobenzoxazole, 5,6-dimethylbenzoxazole, 5-phenylbenzoxazole, 5-hydroxybenzoxazole, 5-methoxybenzoxazole, 5-ethoxybenzoxazole, 6-dialkylaminobenzoxazole, 5-carboxybenzoxazole, 5-sulfobenzoxazole, 5-sulfonamidobenzoxazole, 5- $\beta$ -carboxyvinylbenzoxazole etc.), those of the naphthoxazole series (for example naphtho(1,2-d)oxazole, naphtho(2,1-d)oxazole or naphtho(2,3-d)oxazole), those of the imidazole series (for example 1-methylimidazole, 1-ethyl-4-phenylimidazole, 1-butyl-4,5-dimethylimidazole etc.), those of the benzimidazole series (for example 1-methylbenzimidazole, 1-butyl-4-methylbenzimidazole, 1-ethyl-5,6-dichlorobenzimidazole, 1-ethyl-5-trifluoromethylbenzimidazole etc.), those of the naphthimidazole series (for example 1-methylnaphtho(1,2-d)imidazole or 1-ethyl-naphtho(2,3-d)imidazole), those of the 3,3-dialkyldolnenine series (for example 3,3-dimethylindolenine, 3,3,5-trimethylindolenine, 3,3-dimethyl-5-methoxyindolenine etc.), those of the 2-pyridine series (for example pyridine, 3-methylpyridine, 4-methylpyridine, 5-methylpyridine, 6-methylpyridine, 3,4-dimethylpyridine, 3,5-dimethylpyridine, 3,6-dimethylpyridine, 4,5-dimethyl-

pyridine, 4,6-dimethylpyridine, 4-chloropyridine, 5-chloropyridine, 6-chloropyridine, 3-hydroxypyridine, 4-hydroxypyridine, 5-hydroxypyridine, 6-hydroxypyridine, 3-phenylpyridine, 4-phenylpyridine, 6-phenylpyridine etc.), those of the 4-pyridine series (for example 2-methylpyridine, 3-methylpyridine, 2,3-dimethylpyridine, 2,5-dimethylpyridine, 2,6-dimethylpyridine, 2-chloropyridine, 3-chloropyridine, 2-hydroxypyridine, 3-hydroxypyridine etc.), those of the 2-quinoline series (for example quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, 5-oxo-5,6,7,8-tetrahydroquinoline etc.), those of the 4-quinoline series (for example quinoline, 6-methoxyquinoline, 7-methylquinoline, 8-methylquinoline etc.), those of the isoquinoline series (for example isoquinoline or 3,4-dihydroisoquinoline), those of the thiazoline series (for example thiazoline, 4-methylthiazoline etc.), as well as those of the pyrroline, tetrahydropyridine, thiadiazole, oxadiazole, pyrimidine, triazine or benzthiazine series. The heterocyclic rings and aryl groups may be further substituted in any way desired, for example by further alkyl groups with preferably not more than 3 C-atoms, such as methyl or ethyl, halogen such as chlorine, bromine or iodine or the trifluoromethyl group, hydroxyl, alkoxy with preferably not more than 3 C-atoms, such as methoxy or ethoxy, hydroxalkyl, alkylthio, aryl, such as phenyl, or aralkyl such as benzyl, amino, substituted amino and so on.

For example, the following compounds are suitable:



3,810,760

**15**

B7.....



B8.....



B9.....

**16**

ClO4(-)

B10.....



B11.....



B12.....



C2H5-SO4(-)

B13.....



B14.....



B15.....



B16.....



B17.....



J(-)

B18.....



3,810,760

17



18

J(→)

Tos(→)

Tos(→)

Cl(→)

Tos(→)

Tos(→)

Tos(→)

Cl(→)

Tos(→)

Tos(→)

C<sub>2</sub>H<sub>5</sub>—SO<sub>4</sub>(→)

3,810,760

19



20

J(-)

C<sub>2</sub>H<sub>5</sub>-SO<sub>4</sub>(-)C<sub>2</sub>H<sub>5</sub>-SO<sub>4</sub>(-)C<sub>2</sub>H<sub>5</sub>-SO<sub>4</sub>(-)

J(-)

J(-)

C<sub>2</sub>H<sub>5</sub>-SO<sub>4</sub>(-)C<sub>2</sub>H<sub>5</sub>-SO<sub>4</sub>(-)

Br(-)



The dyes of Formulae II-V are obtained by condensation of 2-methyl quaternary salts of heterocyclic bases or ketomethylene compounds with the corresponding aldehydes in solvents such as alcohol, pyridine or glacial

The mono-, tri- and pentamethine cyanines of Formula I can be synthesized by known methods, see, for example, F. M. Hamer: The Cyanine Dyes and Related Compounds (1964).

acetic acid with the addition of a base such as triethylamine or piperidine.

We now describe in detail the preparation of the compounds B 15 and B 23. The other compounds are obtained in a similar way.

Compound B15

2.0 g. of 1,3-diethyl-thiobarbituric acid were refluxed for 5 minutes with 3.7 g. 3,5-diido-4-hydroxy-benzaldehyde in 30 ml. glacial acetic acid with the addition of 3 ml. piperidine. The mixture was cooled, the dye removed by suction and recrystallized from methanol. 3.6 g. of the dye of M.P. 248° C. (decomposed) were obtained.

Compound B23

4.0 g. of 2-methyl-3-ethyl-benzoselenazole tosylate was heated on a steam bath for 15 minutes with 3.7 g. 3,5-diido-4-hydroxybenzaldehyde in 50 ml. alcohol with addition of 2 ml. triethylamine. After only a short time the dye precipitates. The mixture was cooled, the dye removed by suction, washed with alcohol and recrystallized from dimethylformamide. 3.7 g., M.P. 237° C. (decomposed).

The dyes of Formula II may also, in the case of this preparation, be present in the quinoid form as a result of the acid corresponding to the anion being split off (cf. F. M. Hamer: The Cyanine Dyes and Related Compounds, 1964, page 592). This is, however, without importance in relation to their effectiveness for the purpose of the invention.

(C) Merocyanines of the general formula:



wherein

R<sup>16</sup>=(1) a saturated or unsaturated aliphatic group with preferably not more than 6 C-atoms, which may be substituted, for example, with halogen or phenyl, hydroxyl, amino, carboxyl, sulfo, sulfamoyl, carbamoyl, carboxyalkyl, alkoxy carbonyl, sulfato or thiosulfato groups, (2) cycloalkyl such as cyclohexyl; or (3) aryl, especially a group of the phenyl series;

R<sup>17</sup>=CN, —CO—R<sup>9</sup>, —CO—N(R<sup>9</sup>)<sub>2</sub>, —COOR<sup>9</sup>;

R<sup>18</sup>=R<sup>9</sup>, —O—R<sup>9</sup>, —N(R<sup>9</sup>)<sub>2</sub>,



R<sup>17</sup> and R<sup>18</sup> may also represent the ring members required for completing an iso- or heterocyclic ketomethylene ring; these are the rings usual in cyanine chemistry such as those of the rhodanine series like 3-ethylrhodanine, 3-allylrhodanine, 3-cyclohexylrhodanine, those of the 2-thio-2,4-oxazolidindione series like 3 - ethyl-2-thio-2,4-oxazolidindione, those of the thiohydantoine series like 1,3-dimethyl-2-thiohydantoine, 1-methyl - 3 - phenyl-2-thiohydantoine, those of the barbituric acid or thiobarbituric acid series like 1,3-diethylthiobarbituric acid, 1,3-diphenylthiobarbituric acid, those of the isoxazolone, oxindole, 2-thio-2,5-thiazolidindione, 2,4 - imidazolidindione series or the ketomethylene compounds indicated by the following structural formulae:



R<sup>19</sup>=hydrogen, alkyl with up to 4 C-atoms, hydroxyl, alkoxy with up to 4 C-atoms, such as methoxy or ethoxy, or aryl such as phenyl;

R<sup>9</sup>=the meaning given above;

X<sub>2</sub>=oxygen or sulfur;

n<sub>2</sub>=0, 1 or 2;

m=4, 5 or 6;

Q<sub>1</sub>=the ring members required for completing a 5- or 6-membered heterocyclic ring; the heterocyclic group can contain a fused benzene or naphthalene ring and further substituents; these include the heterocyclics usual in cyanine chemistry such as those of the thiazole series (for example, thiazole, 4-methylthiazole, 5 - methylthiazole, 4,5-dimethylthiazole, 4-phenylthiazole, 5-phenylthiazole, 4,5-diphenylthiazole etc.), those of the benzothiazole series (for example, benzothiazole, 4 - chlorobenzothiazole, 5-chlorobenzothiazole, 6 - chlorobenzothiazole, 7-chlorobenzothiazole, 6-bromobenzothiazole, 5-iodobenzothiazole, 6-iodobenzothiazole, 4 - methylbenzothiazole, 5-methylbenzothiazole, 6-methylbenzothiazole, 5,6-dimethylbenzothiazole, 4-phenylbenzothiazole, 5-phenylbenzothiazole, 6-phenylbenzothiazole, 5 - hydroxybenzothiazole, 6-hydroxybenzothiazole, 4 - methoxybenzothiazole, 5-methoxybenzothiazole, 6-methoxybenzothiazole, 5 - ethoxybenzothiazole, 6-ethoxybenzothiazole, 5,6-dimethoxybenzothiazole, 5,6-methylenedioxybenzothiazole, 5 - diethylaminobenzothiazole, 6-diethylaminobenzothiazole, 5-carboxybenzothiazole, 5-sulfobenzothiazole, tetrahydrobenzothiazole, 7-oxotetrahydrobenzothiazole etc.), those of the naphthothiazole series (for example, naphtho(1,2-d)thiazole, naphtho(2,1-d)thiazole, 5 - methoxynaphtho(2,1-d)thiazole, 5-ethoxynaphtho(2,1-d)thiazole, 7-methoxynaphtho(2,1-d)thiazole, 8 - methoxynaphtho(1,2-d)thiazole etc.), those of the selenazole series (for example, 4-methylselenazole or 4-phenylselenazole), those of the benzoselenazole series (for example, benzoselenazole, 5-chlorobenzoselenazole, 5,6-dimethylbenzoselenazole, 5-hydroxybenzoselenazole, 5-methoxybenzoselenazole, tetrahydrobenzoselenazole, etc.), those of the naphthoselenazole series (for example, naphtho(1,2-d)selenazole or naphtho(2,1-d)selenazole), those of the oxazole series (for example, oxazole, 4-methyloxazole, 4-phenyloxazole, 4,5-diphenyloxazole etc.), those of the benzoaxazole series (for example, benzoaxazole, 5-chlorobenzoaxazole, 6-chlorobenzoaxazole, 5,6 - dimethylbenzoaxazole, 5-phenylbenzoaxazole, 5 - hydroxybenzoaxazole, 5-methoxybenzoaxazole, 5-ethoxybenzoaxazole, 6-dialkylaminobenzoaxazole, 5 - carboxybenzoaxazole, 5 - sulfonylbenzoaxazole, 5 - sulfonamidobenzoaxazole, 5-β-carboxyvinylbenzoaxazole etc.), those of the naphthoxazole series (for example, naphtho(1,2 - d)oxazole, naphtho(2,1-d)oxazole or naphtho(2,3-d)oxazole), those of the imidazole series (for example, 1-methylimidazole, 1-ethyl-4-phenylimidazole, 1-butyl - 4,5 - dimethylimidazole etc.), those of the benzimidazole series (for example, 1-methylbenzimidazole, 1 - butyl-4-methylbenzimidazole, 1-ethyl-5,6-dichlorobenzimidazole, 1-ethyl-5-trifluoromethylbenzimidazole etc.), those of the naphthimidazole series (for example, 1-methylnaphtho(1,2-d)imidazole or 1-ethylnaphtho(2,3-d)imidazole), those of the 3,3-dialkylindolenine series (for example, 3,3-dimethylindolenine, 3,3,5 - trimethylindolenine, 3,3 - dimethyl-5-methoxyindolenine etc.), those of the 2-pyridine series (for example, pyridine, 3-methylpyridine, 4-methylpyridine, 5-methylpyridine, 6 - methylpyridine, 3,4-dimethylpyridine, 3,5 - dimethylpyridine, 3,6 - dimethylpyridine, 4,5-dimethylpyridine, 4,6-dimethylpyridine, 4-chloropyridine, 5-chloropyridine, 6 - chloropyridine, 3-hydroxypyridine, 4-hydroxypyridine, 5-hydroxypyridine, 6-hydroxypyridine, 3-phenylpyridine, 4-phenylpyridine, 6-phenylpyridine, etc.), those of the 4-pyridine series (for example, 2-methylpyridine, 3-methylpyridine, 2,3-dimethylpyridine, 2,5 - dimethylpyridine, 2,6-dimethylpyridine, 2-chloropyridine, 3 - chloropyridine, 2-hydroxypyridine, 3-hydroxypyridine etc.), those

of the 2-quinoline series (for example, quinoline, 3-methylquinoline, 5 - methylquinoline, 7 - methylquinoline, 8-methylquinoline, 6-chloroquinoline, 8-chloroquinoline, 6-methoxyquinoline, 6 - ethoxyquinoline, 6-hydroxyquinoline, 8-hydroxyquinoline, 5 - oxo-5,6,7,8-tetrahydroquinoline etc.), those of the 4-quinoline series (for example, quinoline, 6-methoxyquinoline, 7-methylquinoline, 8-methylquinoline etc.), those of the isoquinoline series (for example, isoquinoline or 3,4-dihydroisoquinoline), those of the thiazoline series (for example, thiazoline, 4-methylthiazoline etc.), as well as those of the pyrroline, tetrahydropyridine, thiadiazole, oxadiazole, pyrimidine, triazine or benzthiazine series.

The heterocyclic rings can be additionally substituted in any way desired, for example, with further alkyl groups with preferably not more than 3 C-atoms, such as methyl or ethyl, halogen such as chlorine, iodine or bromine, trifluoromethyl, hydroxy, alkoxy with preferably not more than 3 C-atoms, such as methyl or ethyl, halogen such as chlorine, iodine or bromine, trifluoromethyl, hydroxyl, alkoxy with preferably not more than 3 C-atoms, such as methoxy or ethoxy, hydroxylalkyl, alkylthio, aryl such as phenyl, or aralkyl such as benzyl, amino, substituted amino and so on.

For example, the following compounds are suitable:









The light-sensitive layers preferably contain at least one sensitizer in an amount of 10-300 mg./m.<sup>2</sup>, one or more of the guanidine derivatives in an amount of 10-500 mg./m.<sup>2</sup> and one or more image-producing reducing agents in an amount of 0.02-0.5 g./m.<sup>2</sup>. These concentration ranges have proved suitable although, of course, it is also possible to operate outside these concentrations.

70 75

The concentration largely depends on the requirements of the particular reproduction process.

Particularly suitable combinations of the sensitizers with the image-producing reducing agents and the guanidine derivatives of the inventions can be found by simple tests. In order to achieve optimum results the choice of solvent and of the binding agent used in the preparation

of the light-sensitive emulsion is also of some importance. The best combination of components for each purpose can be discovered by the usual experiments familiar to anyone skilled in the art.

In order to prepare the light-sensitive coating, guanidine derivatives, sensitizers and image-producing reducing agents can be suspended or dissolved in solvents and, mixed with a binding agent, coated onto the layer support.

In the preparation of the light-sensitive casting solution, it is advantageous to dissolve the components in the solvent in the order—sensitizer-reducing agent-guanidine derivative. This applies particularly in the use of sensitizers that are attacked by any strongly basic medium and with which worse results can be obtained on adding the components in the order sensitizer-guanidine derivative-reducing agent or guanidine derivative-sensitizer-reducing agent.

As binding agents for the light-sensitive emulsion the usual natural or synthetic film-forming polymers are suitable such as proteins, especially gelatin, cellulose derivatives, especially cellulose ethers, cellulose esters or carboxymethylcellulose, alginic acid and its derivatives, starch ethers or galactomannans, as well as polyvinylalcohol, polyvinylpyrrolidone, polyvinylchloride, copolymers of vinylchloride and vinylacetate, polyvinylacetate or completely or partly hydrolyzed polyvinylacetate or copolymers of vinylacetate, mixed polymers of acrylonitrile and acrylamide, polyacrylic acid esters, polymethacrylic acid esters, polyethylene etc.

The light-sensitive layer can be used as self-supporting films or applied to a layer support. Suitable supports are, for example, paper, especially baryta-coated or laminated paper. Cellulose esters, for example cellulose triacetate, polyesters, especially those based on ethyleneterephthalate, glass etc.

The image-receiving material consists preferably of an image-receiving layer which is applied to a suitable support. The same substances are, in general, suitable both as binding agents for the image-receiving layer and also the supports. Such substances have been described above as binding agents for the light-sensitive material.

In choosing a binder for the light-sensitive layer and the image-receiving layer, care should be taken that the coatings do not adhere together on heating. These difficulties, are, however, known from other transfer processes such as the silver salt diffusion process or the heat development process and can be overcome without trouble using the experience gained in these known fields.

The image-receiving layer contains compounds that, under the conditions of the process of the invention, should not be sensitive or should be only very slightly sensitive to light and react with the transferred image-producing compounds to form colored products. A number of compounds have proved suitable for this purpose. These compounds belong chemically to the most different classes so that a uniform classification is not possible. Suitable compounds and suitable combinations of an image-producing compound which is incorporated in the light-sensitive layer coating, and of the reaction partner for the reaction in the image-receiving layer which yields the image dye, can, however, be easily found by simple laboratory tests customarily employed in the art. Thus, the two reaction partners must react, on brief heating for a few seconds at a temperature of from 80 to 200° C., to give a stable image dye. A second test is then required for the selection of suitable image-producing compounds in order to find out whether the image-producing compound reacts rapidly enough on exposure in the presence of the guanidine derivative and the sensitizer so that heating of the mixture thus exposed together with the reaction partner of the image-receiving emulsion produces no more colored compound.

As reaction partner in the image-receiving layer for the image-producing compounds, heavy metal compounds are suitable, especially of metals of Groups IIIa, IVa and Va and Groups Ib, IIb, VIIb and VIII of The Periodic

Table of the Elements, for example, compounds of the heavy metals: cadmium, mercury, iron, cobalt, nickel, copper, silver, gold, bismuth or thallium. Salts of these metals with long chain aliphatic carboxylic acids are particularly suitable, such as nickel stearate, cobalt palmitate, iron stearate, the addition compound of bismuth nitrate with amines, for example triethanolamine. Silver compounds have proved particularly suitable which, under the conditions of the copying process of the invention, are largely insensitive to light, for example the silver salts described in U.K. patent specification No. 1,111,492 of aliphatic carboxylic acids with a thioether group or silver salts of long chain fatty acids, such silver behenate, silver palmitate, silver stearate etc.

With the use of the above mentioned heavy metal compounds brown to black copies are generally obtained. The image consists of the metal in question and/or a reaction product of the transferred image-producing compound.

The image-receiving layers may further contain additives that have a favourable effect on the color tone, contrast, stability etc. of the copy. Such image-receiving layers are already known and described, for example, in DAS 895,101, 1,003,577, 1,159,758, 1,004,043 and 1,165,410, in Netherlands Pat. No. 277086 and in Belgian Pat. Nos. 614064 and 609057.

The image-receiving layers may also contain white pigments, such as zinc oxide or silicon dioxide or titanium dioxide as fillers to improve the whiteness and influence the adhesive tendency and terpene resins and organic acids to improve the storage stability. Such image-receiving coatings are described in U.S. Pat. Nos. 3,074,809 and 3,107,174.

The color tone of the resulting images can be influenced, for example, by compounds of the 1-(2H)-phthalazinone series; such toners are described in U.S. Pat. Nos. 3,080,254 and 3,446,648.

Phthalimide and its derivatives can also be used for this purpose. Additives which accelerate the reduction reaction in the image-receiving layer have also been found advantageous. For example, sterically hindered phenols, such as 2,6-di-tert-butyl-p-cresol, are suitable for this purpose. Such compounds are described in U.S. Pat. No. 3,218,166. Moreover the tone and density of the image can be improved by certain metal salts, such as copper-II-stearate. Such metal ion image-intensifiers and their use are described in DAS 1,572,209.

For exposure of the light-sensitive layer coatings of the invention, light sources customarily employed in the art, such as mercury lamps, iodine quartz lamps or incandescent lamps can be used. The spectral sensitivity of the light-sensitive material depends on the nature of the sensitizing dye used and on the combination of dye and reducing agent.

The exposure can be carried out by contact, optical or reflex methods.

The transfer of the image-producing compounds from the unexposed areas of the light-sensitive emulsions to the image-receiving coating occurs at temperatures of from 80 to 200° C. The heating can be brought about, for example, by conducting the exposed light-sensitive layer while in contact with the image-receiving layer over hot plates or rollers or by uniform exposure with infrared light. The most favourable temperature and heating time of course depends on the nature of the image-producing compound; it can be discovered by a few simple experiments.

According to one modification of the material of the invention, it is also possible to combine the image-receiving layer and the light-sensitive layer on on layer support. In this case it is necessary to use a transparent support to which first the image-receiving layer, for example a layer which contains silver behenate dispersed in a copolymer of styrene and isobutylene, is applied and to apply the light-sensitive layer on to the image-receiving layer, for

example an ethyl-cellulose coating which contains the sensitizer, the guanidine derivative and the reducing agent.

By combination of the photo-reducible dyes for use in accordance with the invention with those described, for example, in the U.S. Pat. No. 3,094,417 such as erythrosin, 5 the sensitivity of these light-sensitivity layers can be increased or widened to other regions of the spectrum in a way that depends on the absorption of the sensitizers. In such combinations also, the addition of the guanidine derivatives of the invention yields an increase in the 10 sensitivity.

#### EXAMPLE 1

##### Light-sensitive material:

A semitransparent paper support was coated with the 15 following solution:

| Dye according to Table 2             | mg | 6     |
|--------------------------------------|----|-------|
| 2-(p-chlorophenyl)-acetoacetonitrile | mg | 125   |
| o-Tolylbiguanide                     | mg | 30    |
| Ethylacetate                         | ml | 70 20 |
| Methanol, and                        | ml | 5     |
| Ethylcellulose                       | g  | 2.5   |

The layer was dried in the usual way. For comparison, a light-sensitive coating not containing o-tolylbiguanide was prepared in the same way.

The image-receiving material was prepared by grinding

| Mixture of silver behenate and behenic acid (molar ratio 1:1) | G.    | 2.1 | 30 |
|---------------------------------------------------------------|-------|-----|----|
| Terpene resin                                                 | 1.66  |     |    |
| 1-(2H)-phthalazinone                                          | 0.86  |     |    |
| Zinc oxide                                                    | 4.8   |     |    |
| Silica gel                                                    | 0.56  |     |    |
| 2,6-di-tert.-butyl-4-methylphenol                             | 0.37  | 35  |    |
| Tetrachlorophthalic acid anhydride                            | 0.034 |     |    |
| 8% ethylmethacrylate solution in pentanone-3                  | 15.0  |     |    |
| 1.5% polyvinylacetate solution in butylacetate                | 80.0  |     |    |
| Butylacetate                                                  | 30.0  |     |    |

in a ball mill, coating on to a paper support and drying. The dried layer contained about 0.2 g. silver per m.<sup>2</sup> in the form of the silver salt.

##### Treatment

The light-sensitive material was exposed behind a  $\sqrt{2}$  step wedge for 5 minutes to 1000 watt iodine quartz lamp at a distance of 30 cm.

Thereupon the exposed layer was brought into contact with the image-receiving layer and heated for 10 seconds at a temperature of 125° C. or treated in a commercial heat-developing apparatus. Brownish-black copies of the wedge were obtained. The increase in sensitivity obtained by the addition of the guanidine derivative can be seen from the difference between the step numbers of the sample and of the guanidine-free control sample. The results are shown in the following table:

TABLE 2

| Dye number | $\sqrt{2}$ -wedge steps of the sample |           |
|------------|---------------------------------------|-----------|
|            | With 1                                | Without 1 |
| A3         | 2                                     | 0         |
| A5         | 3                                     | 0         |
| A7         | 4                                     | 0         |
| A8         | 8                                     | 2         |
| A12        | 8                                     | 0         |
| A13        | 6                                     | 0         |
| A15        | 6                                     | 0         |
| A16        | 4                                     | 0         |
| A17        | 7                                     | 1         |
| A19        | 7                                     | 1         |
| A28        | 3                                     | 0         |
| A27        | 6                                     | 0         |
| A28        | 8                                     | 1         |
| A31        | 3                                     | 0         |
| A32        | 8                                     | 1         |
| A33        | 11                                    | 3         |
| A35        | 5                                     | 0         |
| A36        | 7                                     | 1         |
| A37        | 3                                     | 0         |

TABLE 2—Continued

| Dye number | $\sqrt{2}$ -wedge steps of the sample |           |
|------------|---------------------------------------|-----------|
|            | With 1                                | Without 1 |
| B4         | 4                                     | 0         |
| B5         | 2                                     | 0         |
| B9         | 3                                     | 0         |
| B10        | 3                                     | 0         |
| B11        | 5                                     | 0         |
| B13        | 3                                     | 0         |
| B14        | 4                                     | 0         |
| B15        | 2                                     | 0         |
| B16        | 5                                     | 0         |
| B23        | 6                                     | 0         |
| B24        | 5                                     | 0         |
| B25        | 3                                     | 0         |
| B26        | 1                                     | 0         |
| B28        | 1                                     | 0         |
| B29        | 3                                     | 0         |
| B30        | 5                                     | 0         |
| B32        | 7                                     | 1         |
| B33        | 7                                     | 1         |
| B36        | 2                                     | 0         |
| B37        | 2                                     | 0         |
| C1         | 3                                     | 0         |
| C14        | 4                                     | 0         |
| C15        | 2                                     | 0         |
| C18        | 2                                     | 0         |
| C26        | 4                                     | 0         |
| C27        | 3                                     | 0         |
| C28        | 6                                     | 0         |
| C29        | 3                                     | 0         |
| C30        | 3                                     | 0         |
| C31        | 3                                     | 0         |
| C32        | 5                                     | 0         |
| C38        | 7                                     | 0         |

<sup>1</sup> o-Tolylbiguanide additive.

#### EXAMPLE 2

A light-sensitive material was prepared as in Example 1, using a solution of the following composition:

|                                                  |    |       |
|--------------------------------------------------|----|-------|
| Dye according to Table 3                         | mg | 6.0   |
| Acylacetonitrile derivative according to Table 3 | mg | 125.0 |
| Guanidine derivative according to Table 3        | mg | 30.0  |
| Ethylcellulose                                   | g  | 2.5   |
| Ethyl acetate                                    | ml | 75.0  |

The same image-receiving material was used as in Example 1. The treatment was as described in Example 1. The results of the sensitometric tests are shown in the following table:

TABLE 3

| Dye number | Acyl-aceto-nitrile No. | Number of $\sqrt{2}$ -wedge steps |    |
|------------|------------------------|-----------------------------------|----|
|            |                        | Guanidine derivative              |    |
| A32        | 7                      | 1,3-diphenylguanidine             | 6  |
| A32        | 7                      | 1,3-di-o-tolylguanidine           | 7  |
| B33        | 7                      | do                                | 8  |
| B33        | 7                      | 1,3-diphenylguanidine             | 8  |
| A33        | 7                      | do                                | 10 |
| A19        | 7                      | do                                | 6  |
| C38        | 7                      | do                                | 6  |
| B23        | 7                      | do                                | 6  |
| A12        | 7                      | 1,3-di-o-tolylguanidine           | 6  |
| A12        | 7                      | 1,3-diphenylguanidine             | 8  |
| A32        | 5                      | o-tolylbiguanidine                | 7  |
| A32        | 16                     | do                                | 6  |
| B33        | 14                     | do                                | 7  |

#### EXAMPLE 3

A light-sensitive material was prepared by dipping a semi-transparent paper support into a solution of the following composition and drying at room temperature:

|                                      |    |       |
|--------------------------------------|----|-------|
| Dye as in Table 4                    | mg | 6.0   |
| 2-(p-chlorophenyl)-acetoacetonitrile | mg | 125.0 |
| o-Tolylbiguanide                     | mg | 30.0  |
| Ethylcellulose                       | g  | 2.5   |
| Ethyl acetate                        | ml | 70.0  |
| Methanol                             | ml | 5.0   |

The light-sensitive material was exposed in reflex in contact with an original sheet written on both sides in a commercial reflex copying device provided with a 1000 w. iodine quartz lamp as light source. The exposed layer was then heated in contact with an image-receiving layer for

10 seconds at 130° C. A black copy of the original in the image-receiving layer was obtained. The image-receiving material was prepared in the following way;

|                         | G.   | 5 |
|-------------------------|------|---|
| Zinc oxide              | 6.0  |   |
| Calcium carbonate       | 6.0  |   |
| Silver stearate         | 1.5  |   |
| Phthalimide             | 0.6  |   |
| Stearic acid            | 0.2  |   |
| Polyvinylbutyral        | 1.0  |   |
| Cellulose acetobutyrate | 2.0  |   |
| Ethyl acetate           | 60.0 |   |

was ground overnight in a ball mill and after adding 1.5 g. 2,6-dicyclohexyl-p-cresol applied to a paper support and dried. The silver applied amounted to 0.3 g./m.<sup>2</sup> in the form of the silver salt. The results of sensitometric tests are given in the following table. As reflex copying time the minimum exposure required for the production of saturated blacks and clear whites is quoted. The spectral sensitivity was determined by exposing through a set of color filters of the following transmissivities:

350 nm., 390 nm., 405 nm., 435 nm., 480 nm., 505 nm., 515 nm., 540 nm., 550 nm., 570 nm., 590 nm., 605 nm.

The light-sensitive material was exposed for 5 to 30 minutes, depending on the dye, behind the filters to an iodine quartz lamp of 1000 watts at a distance of 30 cm. Then the exposed material was placed in contact with the image-receiving layer described in Example 3 and treated in a commercial heat developing apparatus.

TABLE 4

| Dye number | Reflex copying time/sec. | Spectral sensitivity/nm. |
|------------|--------------------------|--------------------------|
| A32        | 12                       | 405, 480                 |
| A27        | 25                       | 405, 480                 |
| A13        | 15                       | 405, 480                 |
| A12        | 13.5                     | 405, 480                 |
| A15        | 18                       | 405, 435, 480            |
| A36        | 15                       | 480                      |
| A19        | 13.5                     | 405, 480                 |
| A8         | 10                       | 405, 480, 515            |
| A26        | 40                       | 540                      |
| A37        | 40                       | 480                      |
| A33        | 4.5                      | 405, 480, 505, 540       |
| B4         | 30                       | -----                    |
| B16        | 20                       | 480, 505, 515            |
| B11        | 12                       | 540, 590, 605            |
| B9         | 50                       | 590, 605                 |
| B32        | 15                       | 590, 605                 |
| B33        | 10.5                     | 540, 590, 605            |
| B23        | 18                       | 590, 605                 |
| B30        | 30                       | 590, 605                 |
| B41        | 22                       | -----                    |
| B43        | 35                       | -----                    |
| B49        | 35                       | -----                    |
| C38        | 20                       | 480, 515                 |
| C26        | 30                       | 480, 515                 |

In tests with light-sensitive layers which had been prepared in a similar way but without addition of the biguanide, no copies with clear whites were obtained or only copies with poor contrast and much lower sensitivity.

#### EXAMPLE 4

By combining suitable dyes it is possible to produce emulsion coatings sensitive to several regions of the spectrum. For this purpose, erythrosine, which is sensitive at 540 nm., can be employed with advantage as a component dye. In order to do this, for example, the dyes, 2-(p-chlorophenyl)-acetoacetonitrile and o-tolylbiguanide were added, in the amounts given in Table 5, to the casting solution which contained 2.5 g. ethylcellulose in 75 ml. ethylacetate. The subsequent treatment was carried out as in Example 3.

TABLE 5

C=2-(p-chlorophenyl)-acetoacetonitrile (mg.)  
T=o-tolylbiguanide (mg.)  
R=reflex copying time (sec.)  
S=spectral sensitivity (nm.)

|                                                 | Mg. Dye number | C  | T    | R                  | S |
|-------------------------------------------------|----------------|----|------|--------------------|---|
| 4 mg. A32 plus 4 mg. B11                        | 180            | 60 | 12   | 405, 480, 515, 590 |   |
| 4 mg. A32 plus 4 mg. A12                        | 180            | 60 | 15   | 405, 480, 515, 590 |   |
| 4 mg. erythrosine plus 4 mg. A8                 | 180            | 30 | 12   | 405, 480, 515, 540 |   |
| 6 mg. erythrosine plus 6 mg. A32                | 240            | 45 | 18   | 405, 480, 515, 540 |   |
| 3 mg. erythrosine plus 3 mg. B33                | 125            | 30 | 10   | 540, 590, 605      |   |
| 4 mg. erythrosine plus 4 mg. B32                | 180            | 60 | 13.5 | 540, 590, 605      |   |
| 4 mg. erythrosine plus 4 mg. B23                | 180            | 30 | 15   | 540, 590, 605      |   |
| 4 mg. B33 plus 4 mg. B11                        | 180            | 60 | 15   | 540, 590, 605      |   |
| 4 mg. B33 plus 4 mg. A12                        | 125            | 30 | 9    | 405, 480, 590, 605 |   |
| 4 mg. B33 plus 4 mg. B16                        | 180            | 60 | 12   | 405, 480, 590, 605 |   |
| 3 mg. B33 plus 3 mg. A32                        | 125            | 30 | 12   | 480, 590, 605      |   |
| 3 mg. B32 plus 3 mg. erythrosine plus 3 mg. A32 | 180            | 45 | 15   | 405, 480, 515-605  |   |
| 4 mg. erythrosine plus 4 mg. B33 plus 4 mg. A32 | 180            | 90 | 9    | 405, 480, 515-605  |   |
| 2 mg. erythrosine plus 2 mg. B32 plus 2 mg. A32 | 125            | 30 | 10.5 | 405, 480, 515-605  |   |
| 4 mg. B11 plus 4 mg. A32 plus 4 mg. erythrosine | 180            | 90 | 9    | 405, 480-550       |   |
| 10 mg. B41 plus 10 mg. B43 plus 10 mg. B49      | 118            | 38 | 15   | -----              |   |

If the guanidine derivative is omitted the layers show a considerable loss of sensitivity and flattening of the gamma value.

What is claimed is:

1. A process for producing photographic images comprising exposing to image-forming light a light-sensitive layer containing an image-producing compound capable of being transferred from said layer and being characterized as readily forming a nontransferable product upon exposure, said exposure being for a time sufficient to form non-transferable portions of said image-producing compound in exposed areas, placing the exposed layer in contact with a receiving layer of material containing a heavy metal compound which reacts with transferred image-producing compound to form colored compounds, heating of the layers in contact with each other at a temperature of between 80-200° C. to transfer the image-forming compound in the unexposed areas to the receiving layer and forming a visible image in the receiving layer, wherein the improvement comprises the image-producing transferable compound is an acylacetonitrile derivative having the following formula:



wherein R<sup>3</sup> represents

alkyl with up to 5 carbon atoms;  
alkoxy with up to 5 carbon atoms;  
aryl or aralkyl;

R<sup>4</sup> represents

aryl or a heterocyclic group of the class consisting of furyl, pridyl or thiienyl;

the said transferable compound is exposed in the presence of a sensitizing dye from the class of the neutrostyryl dyes, the merocyanines or a cyanine dye containing a halogen substituted benzene ring or a heterocyclic ring derived from selenazol and a compound of the guanidine or biguanide series.

2. The process of claim 1, wherein the guanidine derivative has the following formula:



where

70 R<sup>1</sup>=hydrogen or aryl  
R<sup>2</sup>=aryl or a residue of the formula



3. The process of claim 1, wherein the neutrostyryl dye is selected from those having the following formulae:



where  
 $\text{Q} =$



or  
 $\text{R}^5=\text{cyan, } -\text{CO}-\text{R}^9, -\text{CO}-\text{N}(\text{R}^9)_2, -\text{COOR}^9$   
 $\text{R}^6=\text{R}^9 \text{ or } -\text{O}-\text{R}^9, -\text{N}(\text{R}^9)_2$

$\text{R}^5$  and  $\text{R}^6$  together can also represent the ring members necessary for completing an iso- or heterocyclic ketomethylene ring;

$\text{R}^7=\text{hydrogen or nitro}$

$\text{R}^8=\text{hydrogen, } -\text{O}-\text{R}^9, -\text{S}-\text{R}^9 \text{ or } -\text{N}(\text{R}^9)_2$

$\text{R}^9=\text{a saturated or olefinically unsaturated aliphatic group}$

$\text{Z}^1, \text{Z}^2=\text{hydrogen, alkyl or alkoxy carbonyl; } \text{Z}^1 \text{ and } \text{Z}^2$  can also represent methylene groups required to complete a 5- or 6-membered ring

$n=0, 1 \text{ or } 2$

$\text{X}=\text{oxygen or sulfur.}$

4. The process of claim 1, wherein the halogen and/or selenium containing polymethine dye is selected from those having the following formulae:



where

$\text{Hal}=\text{Cl, Br or I}$

$\text{R}^{10}=(1) \text{ a saturated or unsaturated aliphatic group,}$   
 $(2) \text{ cycloalkyl or (3) aryl}$

$\text{R}^{11}=\text{hydrogen, alkyl, aryl or cycloalkyl}$

$\text{R}^{12}, \text{R}^{13}=\text{hydrogen or hydroxyl, where however at least one of the group stands for hydroxyl}$

$\text{R}^{14}=\text{hydrogen, alkyl or alkoxy, halogen, trifluoromethyl or aryl}$

5  $\text{R}^{15}=\text{aryl or a heterocyclic ring}$

$\text{X}_1=\text{the ring members required for completing a benzene or naphthalene ring which contains—if Y is different from Se—at least one halogen or a trifluoromethyl group}$

10  $\text{Z}^3, \text{Z}^4=\text{hydrogen, alkyl or alkoxy carbonyl; } \text{Z}^3 \text{ and } \text{Z}^4$  can also stand for methylene groups required to complete a 5- or 6-membered ring

$\text{Y}=\text{O, S, Se, } -\text{CH}=\text{CH, } >\text{N-alkyl, } >\text{N-aryl}$

$n=0, 1 \text{ or } 2$

15  $\text{D}=\text{the ring members required to complete an iso- or heterocyclic ketomethylene ring}$

$\text{Q}=\text{the ring members required to complete a 5- or 6-membered heterocyclic ring.}$

5. The process of claim 1, wherein the merocyanine has 20 the following formula:



where

$\text{R}^{16}=(1) \text{ a saturated or unsaturated aliphatic group,}$   
 $(2) \text{ cycloalkyl, (3) aryl}$

$\text{R}^{17}=-\text{CN, } -\text{CO}-\text{R}^9, -\text{N}(\text{R}^9)_2, -\text{COOR}^9$

$\text{R}^{18}=\text{R}^9, \text{O}-\text{R}^9, \text{N}(\text{R}^9)_2 \text{ or}$



$\text{R}^{17}$  and  $\text{R}^{18}=\text{the ring members required for completion of an iso- or heterocyclic ketomethylene ring}$

$\text{R}^{19}=\text{hydrogen, alkyl with not more than 4 C-atoms, hydroxyl, alkoxy with not more than 4 C-atoms or aryl}$

$\text{R}^9=\text{a saturated or olefinically unsaturated aliphatic group,}$

$\text{X}_2=\text{oxygen or sulfur}$

$n_2=0, 1 \text{ or } 2$

$m=4, 5 \text{ or } 6$

$\text{Q}_1=\text{the ring members required for completing a 5- or 6-membered heterocyclic ring.}$

6. A light-sensitive photographic material wherein a transferable light-sensitive compound is converted upon 50 exposure to light to provide a non-transferable product in the exposed areas and a transferable compound in the unexposed areas, said photographic material comprising on a support at least one light-sensitive layer containing as the image-producing transferable compound an acyl-acetonitrile derivative having the following formula:



60 wherein  $\text{R}^3$  represents  
 $\text{alkyl with up to 5 carbon atoms;}$   
 $\text{alkoxy with up to 5 carbon atoms;}$   
 $\text{aryl or aralkyl;}$

$\text{R}^4$  represents

65  $\text{aryl or a heterocyclic group of the class consisting of furyl, pyridyl or thieryl; which transferable compound is transferable at temperature of between 80 and 200}^{\circ}\text{C. to an image-receiving layer;}$

70  $\text{a sensitizer dye from the class of the neutrostyryl dyes, the merocyanines or a cyanine dye containing a halogen substituted benzene ring or a heterocyclic ring derived from selenazol and the neutrostyryl dyes, the merocyanines or a cyanine dye containing a halogen substituted benzene ring or a heterocyclic ring derived from selenazol;}$

and a compound of the guanidine or biguanide series.

7. The light-sensitive photographic material of claim 6, containing a guanidine derivative of the following formula:



where

$\text{R}^1$ =hydrogen or aryl

$\text{R}^2$ =aryl or a group of the formula



8. The light-sensitive photographic material of claim 6, containing a neutrostyryl dye of the following formulae:



where



$\text{R}^5$ =cyan,  $-\text{CO}-\text{R}^9$ ,  $-\text{CO}-\text{N}(\text{R}^9)_2$ ,  $-\text{COOR}^9$

$\text{R}^6$ = $\text{R}^9$  or  $-\text{O}-\text{R}^9$ ,  $-\text{N}(\text{R}^9)_2$

$\text{R}^5$  and  $\text{R}^6$  together can also represent the ring members necessary for completing an iso- or heterocyclic ketomethylene ring

$\text{R}^7$ =hydrogen or nitro

$\text{R}^8$ =hydrogen,  $-\text{O}-\text{R}^9$ ,  $-\text{S}-\text{R}^9$  or  $-\text{N}(\text{R}^9)_2$

$\text{R}^9$ =a saturated or olefinically unsaturated aliphatic group

$\text{Z}^1$ ,  $\text{Z}^2$ =hydrogen, alkyl or alkoxy carbonyl;  $\text{Z}^1$  and  $\text{Z}^2$  can also represent methylene groups required to complete a 5- or 6-membered ring

$n=0, 1$  or  $2$

$\text{X}$ =oxygen or sulfur.

9. The light-sensitive photographic material of claim 6, wherein the halogen and/or selenium containing polymethine dye is selected from those having the following formulae:



$\text{Hal}=\text{Cl, Br or I}$

$\text{R}^{10}=(1)$  a saturated or unsaturated aliphatic group, (2) cycloalkyl or (3) aryl

$\text{R}^{11}$ =hydrogen, alkyl, aryl or cycloalkyl

$\text{R}^{12}$ ,  $\text{R}^{13}$ =hydrogen or hydroxyl, where however at least one of the groups stand for hydroxyl

$\text{R}^{14}$ =hydrogen, alkyl or alkoxy, halogen, trifluoromethyl or aryl

$\text{R}^{15}$ =aryl or a heterocyclic ring

$\text{X}_1$ =the ring members required for completing a benzene or naphthalene ring which contains—if  $\text{Y}$  is different from Se—at least one halogen or trifluoromethyl group

$\text{Z}^3$ ,  $\text{Z}^4$ =hydrogen, alkyl or alkoxy carbonyl groups;  $\text{Z}^3$  and  $\text{Z}^4$  can also stand for methylene groups required to complete a 5- or 6-membered ring

$\text{Y}=\text{O, S, Se, }-\text{CH}=\text{CH}-, >\text{N-alkyl, }>\text{N-aryl}$

$n=0, 1$  or  $2$

$\text{D}$ =the ring members necessary for completing an iso- or heterocyclic ketomethylene ring

$\text{Q}$ =the ring members required for completing a 5- or 6-membered heterocyclic ring.

10. The light-sensitive photographic material of claim 6, wherein the merocyanine has the following formula:



where

$\text{R}^{16}=(1)$  a saturated or unsaturated aliphatic group, (2) cycloalkyl, (3) aryl

$\text{R}^{17}=\text{CN, }-\text{CO}-\text{R}^9, -\text{N}(\text{R}^9)_2, -\text{COOR}^9$

$\text{R}^{18}=\text{R}^9, -\text{O}-\text{R}^9, -\text{N}(\text{R}^9)_2$  or



$\text{R}^{17}$  and  $\text{R}^{18}$ =the ring members required for completing an iso- or heterocyclic ketomethylene ring

$\text{R}^{19}$ =hydrogen, alkyl having up to 4 C-atoms, hydroxyl, alkoxy having up to 4 C-atoms or aryl

$\text{R}^9$ =a saturated or olefinically unsaturated aliphatic group

$\text{X}_2$ =oxygen or sulfur

$n_2=0, 1$  or  $2$

$m=4, 5$  or  $6$

$\text{Q}_1$ =the ring members required for completing a 5- or 6-membered ring.

#### References Cited

#### UNITED STATES PATENTS

- 65 3,619,237 11/1971 Leclair ----- 96—90 R  
 3,458,318 7/1969 Brooks ----- 96—122  
 3,094,417 6/1963 Workman ----- 96—90 R  
 3,690,884 9/1972 Scheibitz et al. ----- 96—77

70 J. TRAVIS, BROWN, Primary Examiner  
 R. L. SCHILLING, Assistant Examiner

U.S. Cl. X.R.

96—77, 90 R